

Jan. 9, 1940.

R. H. CHURCHILL

2,186,667

VULCANIZING FUEL

Filed June 28, 1937



Inventor:

Ralph H. Churchill  
By Chittenden, Niles, Davies & Girschley & Dalton.  
Attest:

## UNITED STATES PATENT OFFICE

2,186,667

## VULCANIZING FUEL

Ralph H. Churchill, Chicago, Ill.

Application June 28, 1937, Serial No. 150,825

8 Claims. (Cl. 44—3)

This invention relates to a fuel and particularly to a fuel for vulcanizing pneumatic rubber tire patches.

This application is a continuation in part of my 5 co-pending application Ser. No. 3,534 filed January 25, 1935.

The vulcanization of tire patches is an old art, the basic principle being the ignition of a fuel supplying a considerable amount of heat, in combination with a means for holding the heat long enough to give proper vulcanization. A mixture of materials comprising powdered aluminum, sulfur, and a small amount of iron has heretofore been suggested for use as a fuel. While this fuel 10 is satisfactory, there is a tendency for the aluminum to cause too high a maximum temperature, the aluminum is expensive, and the resultant product decomposes to form hydrogen sulfide, which is objectionable. 15

As is well known, iron has heretofore been known to be a combustible material under certain conditions. For example, iron filings will burn in pure oxygen and iron will rust readily in the presence of water. It has heretofore been suggested 20 that under certain conditions a heating composition for vulcanizers might be obtained by igniting a mixture of iron filings and sulfur, but under ordinary circumstances such ignition and burning is not easy and therefore iron, except in combination with a vigorously burning metal such as 25 aluminum or magnesium, has not been employed in vulcanizing patches.

This is particularly true with reference to tire vulcanizers, in which the amount of vulcanizing 30 fuel is small and where the fuel is exposed to the atmosphere or to large cooling areas.

It has now been discovered that iron filings 35 may be produced which, when combined with sulfur, will ignite and burn satisfactorily and at the same time will eliminate the disadvantages present when aluminum is used. Such a fuel is likewise less expensive than an aluminum base material.

Normal iron filings, as purchased on the market, 40 are largely made up of two classes of particles. The first type of particles is quite large and the structure thereof visible to the unaided eye. These particles are rough and jagged, but are too large to burn satisfactorily. The second 45 class of particles are very small and their structure is not visible to the naked eye. Under a microscope these particles do not have the rough and jagged appearance of the larger particles, but have a sintered or fused appearance, the individual particles under the microscope resem-

bling small globules or shot-like masses. This type of iron filings will not burn in such manner as to make a satisfactory vulcanizing fuel, even though very fine in size.

It has been discovered, however, that if particles are chosen which do not have a sintered or fused surface and at the same time are in a very fine state of subdivision, a satisfactory vulcanizing fuel may be obtained therefrom.

The term "follicular" is used herein to describe 10 such particles, and designates that the particles have the rough jagged surface which is characteristic of large particles of ordinary filings such as the public is generally acquainted with.

The preferred iron material is produced by 15 grinding, for example with an emery wheel, cast iron piston rings, for example, such rings having a carbon content of 3.8% and a silicon content of 4.34%. The product should be predominantly 20 of particles at least fine enough to pass a 60 mesh screen and preferably above 90% of the product will pass a 150 mesh screen.

Temperature conditions during manufacture of the product must be such as not to produce the fused or sintered particles. With a brittle material such as cast iron piston rings an emery wheel may sometimes be employed in the production of particles, care being taken not to heat them to a sintering or fusing point. However, with certain tough materials such as some of the 30 steels, an emery wheel is unsatisfactory unless great care is taken. In such cases filing may be employed.

To the finely divided iron is added an accelerator, such as sulfur, in the desired proportions. 35 A preferred fuel comprises 75% iron and 25% sulfur. The percentage of sulfur may, however, be varied rather widely, but as it increases the product flames more in burning. A preferred range is from 15—40% sulfur, depending upon the 40 use and the appliances with which used.

Other forms of iron may be used, for example, the product known as iron by hydrogen is quite active. This product is very finely divided, can be ignited with a match and will burn in air alone 45 without an accelerator, but it is preferred to add sulfur or other accelerator to speed up the burning. In this product about 25% sulfur is preferred, with the range from 5—50% being satisfactory.

In some instances it may be desirable to employ in addition to the sulfur an accelerating agent. For example, a .90% carbon steel, ground to 150 mesh, burned satisfactorily when 75 parts were combined with 15 parts of sulfur and 10 55

parts of potassium permanganate, although less permanganate may be used. This steel will burn with red phosphorus alone, although a little permanganate or other rust promoter is preferred.

5 Other accelerators may be used instead of the sulfur. Red phosphorus, for example, is extremely satisfactory. For example, 20% of red phosphorus added to the iron by hydrogen will produce a satisfactory burning fuel.

10 Acidic substances, such as aluminum chloride, zinc chloride and oxidizing substances such as potassium chlorate and sodium nitrate, may likewise be used as accelerators. Certain types of iron require the use of accelerators other than sulfur in order to produce a satisfactory fuel. For example, in certain instances such as above shown, a combination of sulfur and permanganate may produce commercial results where the sulfur alone fails. These acid-forming substances and oxidizing agents may be in general classed as rust promoters, in that all of them promote the oxidation of the iron.

This type of fuel is particularly suitable for use with which is known in the trade as a heavy cup, that is, the fuel is burned in a heavy metallic cup which retains the heat of combustion for a sufficient time to vulcanize the rubber.

25 Steel of about 1.50 carbon content is also satisfactory, for example in combination with sulfur and permanganate in substantially the same proportions as for the 0.90% carbon steel. The 1.50% carbon steel when ground on an emery wheel produces elongated fibres which are particularly desirable in that they will mat and not segregate.

30 The term "accelerator," as used in the claims hereof, excludes aluminum.

A vulcanizing patch is illustrated diagrammatically in the drawing, in which the vulcanizing cup 5 is held in a clamp 1 by the screw 4 against a patch 6 which rests upon the tube 3. The tube is supported by the plate 2 of the clamp. The vulcanizing fuel 13 is placed within the cup

5, wherein it is retained by the flanges 10. A handle 12 may be provided on the cup. In some instances the cup and fuel may be made integrally, the fuel being cemented to the cup.

In manufacturing fuel it is important that the particles be largely of the same size and that no great variation occur therein. For instance, where most of the particles are approximately 200 mesh, substantially none of the particles should be above 150 mesh and substantially none 10 by weight should be below 300 mesh.

What I claim as new and desire to secure by Letters Patent is:

1. A vulcanizing fuel consisting essentially of finely divided iron, substantially all of the particles of which will pass a 60 mesh screen, and a non-metallic accelerator, substantially all of the particles of the iron having a rough jagged surface. 15

2. A product as set forth in claim 1, in which the bulk of the iron particles will pass a 150 mesh screen. 20

3. A vulcanizing fuel as set forth in claim 1, in which the iron is cast iron.

4. A fuel as set forth in claim 1, in which the accelerator is sulfur. 25

5. A fuel as set forth in claim 1, in which the accelerator is a substance of the class consisting of sulfur and phosphorus.

6. A vulcanizing fuel consisting of finely divided iron substantially all of the particles of which will pass a 60 mesh screen, the particles of iron being rough and jagged and free from fused or sintered surfaces, and at least about 33 1/3% of sulfur based upon the amount of iron. 30 35

7. A vulcanizing fuel as set forth in claim 1, in which the iron is cast iron of approximately 3.8% carbon content and 4.34% silicon content.

8. A vulcanizing fuel as set forth in claim 1, in which the accelerator is sulphur and the sulphur is present in an amount from 15% to 40%. 40

RALPH H. CHURCHILL.